

## UNITED STATES PATENT OFFICE.

JOHN HOWARD HELFRICH, OF WHEATON, ILLINOIS.

## COSMETIC.

No Drawing.

Application filed December 4, 1926. Serial No. 152,722.

My invention relates to cosmetics, and more specifically to an improved compact of the type used for dispensing rouge and face powder.

5 The particular embodiment of the process selected for illustration includes the formation of a stiff paste; the fabrication of a compact of substantially the size of the finished article; and the desiccation of the finished compact.

10 According to one illustrative procedure, I take 99 pounds of domestic talc free from silica and mica, 9 pounds of heavy imported chalk, and 15 ounces of yellow ochre. These 15 ingredients are mixed in a powder mill and sifted through a rapid sifter to remove grit.

15 The resulting dry material is then ground into a stiff paste in a mixer. In the mixer I add one hundred cubic centimeters of a 20 fatty-natured emollient, a proper amount of perfume oil to suit the taste of the user, and twelve hundred cubic centimeters of binder to each eighteen pounds of dry material. One emollient I have used is purified 25 water-white mineral oil having a specific gravity of 0.868. In addition to the foregoing, sufficient water is included to make a heavy paste of the whole. The binder is an intimate mixture of water and powdered 30 gum arabic in the ratio of twenty grams of gum arabic to one gallon of water.

35 The paste ingredients are ground in the mixer for from one-half to three-quarters of an hour and molded into compacts of substantially the exact size and shape of the finished product. In the molding operation I form pellets of the paste, each pellet containing a very slight excess of material above that necessary to form the finished compact.

40 A suitable metal plate, with its upper surface slightly roughened, is coated with a non-shrinking and non-absorbing glue and the pellet dropped on the glue. A suitable stamping die is then employed to form the 45 pellet, and the fabricated compact is ready for desiccation.

45 The drying process normally involves standing for about three days in a gentle draft of ordinary atmospheric air. At the 50 end of the drying process the slight top crust accumulating during drying is removed, as by light sand-papering, and the finished product is ready for the user.

The pigment carrying medium in the fin-

ished compact is both plastic to such an extent that the jolting or possible flexure of the supporting plate encountered in ordinary use of the compact will not chip or break it; and sufficiently friable to be capable of use with substantially the same effect as loose 55 powder.

Without further elaboration, the foregoing will so fully explain the gist of my invention, that others may, by applying current knowledge, readily adapt it for use under 60 various conditions of service. Moreover, it is not essential that all the different parts of the invention be employed in conjunction, as certain of them may be advantageously made use of in various combinations and 65 subcombinations.

What I claim is:

1. A compact containing the following ingredients in the following original proportions; a color vehicle, a mineral oil and a binder, in the proportions of 18# of color vehicle to 100 cc. of mineral oil to 1200 cc. of binder, said binder containing originally 20 grams of powdered gum arabic to one gallon of water; said color vehicle comprising domestic talc free from silica, heavy imported chalk, and yellow ochre in the proportions of 99# talc to 9# chalk and 15 oz. yellow ochre.

2. A compact containing the following ingredients in the following original proportions; a color vehicle, a mineral oil and a binder, in the proportions of 18# of color vehicle to 100 cc. of mineral oil, and 1200 cc. of binder, said binder containing originally 20 grams of powdered gum arabic to one gallon of water; said color vehicle comprising domestic talc free from silica, and heavy imported chalk, in the proportions of 99# talc to 9# chalk, and a pigment.

3. A wet-formed compact comprising a color vehicle, a fatty-natured emollient, and a binder, the fatty-natured emollient being not more than 6% of the total solids by weight.

4. A wet-formed compact comprising a color vehicle, a fatty-natured emollient, and a binder, the fatty-natured emollient being not more than 6% of the total solids by weight, and the binder comprising water and a solid not exceeding 2% by weight of the total solids.

5. A wet-formed compact comprising a

color vehicle, a binder, and a fatty-natured emollient, the binder amounting to substantially 0.1% of the total solids, and the emollient amounting to substantially 1% of the total solids.

6. A wet-formed compact containing a color vehicle, and a fatty-natured emollient in the proportion of substantially 99% vehicle and 1% emollient.

10 7. A wet-formed compact containing a color vehicle, a fatty-natured emollient, and a binder, the fatty-natured emollient not exceeding 6% of the total solids by weight, and the binder being sufficient in quantity to produce cohesion substantially equal to that

produced by powdered gum arabic not exceeding 2% of the total solids by weight.

8. A wet-formed compact containing a color vehicle, and a mineral oil, in the proportion of substantially 99% vehicle and 1% oil.

9. A wet-formed compact comprising a binder, a body having substantially the composition resulting from the admixture of ninety-nine pounds of talc with from nine to sixteen pounds of chalk, and substantially one per cent of a fatty-natured emollient.

In testimony whereof, I have signed my name to this specification.

JOHN HOWARD HELFRICH.